

09-21-71

XR

3,607,234

## United States Patent

[11] 3,607,234

[72] Inventors **Takaho Kawawa;**  
**Noburo Shimada; Masaji Kogi; Hidetaro**  
**Nemoto, all of Kawasaki-shi, Japan**

[21] Appl. No. **830,341**

[22] Filed **June 4, 1969**

[45] Patented **Sept. 21, 1971**

[73] Assignee **Nippon Kokan Kabushiki Kaisha**  
**Japan**

[32] Priority **June 8, 1968**

[33] **Japan**

[31] **43/39086**

[56] **References Cited**

**UNITED STATES PATENTS**

|           |         |                   |          |
|-----------|---------|-------------------|----------|
| 2,126,786 | 8/1938  | Laoch et al. .... | 75/96 X  |
| 2,728,681 | 12/1955 | Clipson .....     | 106/97   |
| 3,181,959 | 5/1965  | Raine et al. .... | 106/97 X |
| 3,376,146 | 4/1968  | Mitchell .....    | 106/97   |
| 3,516,821 | 6/1970  | Gerhard .....     | 75/96    |
| 253,158   | 1/1882  | Campbell .....    | 75/96 X  |

**FOREIGN PATENTS**

|         |        |                    |        |
|---------|--------|--------------------|--------|
| 137,925 | 7/1950 | Australia.....     | 106/97 |
| 22,519  | 1910   | Great Britain..... | 106/97 |
| 217,343 | 6/1924 | Great Britain..... | 106/97 |

*Primary Examiner—Allen B. Curtis*  
*Attorney—Flynn & Frishauf*

[54] **STEEL-REFINING COMPOSITION CONTAINING**  
**PORTLAND CEMENT AND FLUORSPAR**  
**6 Claims, 1 Drawing Fig.**

[52] U.S. Cl..... **75/96,**  
**106/97**

[51] Int. Cl..... **C22b 9/10**

[50] Field of Search..... **75/96;**  
**106/97; 148/26**

**ABSTRACT:** A steel-refining agent which is composed of 35% to 65% of Portland cement, 5% to 20% of fluorspar, 20% to 40% of Chamotte powder, 2% to 15% of soda ash, 2% to 15% of a carbon source, which is coke breeze or graphite powder, and further 2% to 15% of borax, wherein more than 50% of mixing particles have a diameter of less than 0.044 mm.

PATENTED SEP 21 1971

3,607,234



STEEL-REFINING COMPOSITION CONTAINING  
PORTLAND CEMENT AND FLUORSPAR

BACKGROUND OF THE INVENTION

This invention relates to a novel steel-refining agent which is added into mold wherein liquid steel is cast and more particularly is cast continuously.

While steel is cast by a bottom pouring method the surface of the molten steel poured into the mould is oxidized by the atmosphere. To avoid this oxidation it is common to cover the surface of the molten steel with straw ash or other heat-insulating material. Also in case of continuous casting, similar problems is brought about. Thus, it is well known that stream of said molten steel poured into a mold from a tundish and surface of said molten steel in said mold is subjected to oxidation caused by the atmosphere. Oxides of iron and deoxidizing element, especially aluminum oxides in case of aluminum killed steel not only tend to clog a nozzle of said tundish but also are entrained in the molten steel as contaminants to degrade the quality of the steel produced. And further, these oxides cause leakage of said molten steel which will bring forth the biggest difficulty of continuous casting process.

SUMMARY OF THE INVENTION

It is an object of this invention to provide a novel steel refining agent which can effectively prevent oxidation of said liquid steel surface in an ordinary mold or a continuous casting mould and can absorb and remove some nonmetallic inclusions such as silica, aluminum or the like when flotation of these inclusions reach the surface of said liquid steel.

BRIEF DESCRIPTION OF THE DRAWING

In the accompanying drawing, a single FIGURE illustrates a cross section of a portion of a continuous casting device to show a relation between the surface of slag formed by the steel refining agent and a pouring nozzle, where the steel-refining agent is added into the continuous casting mould.

DESCRIPTION OF THE PREFERRED EMBODIMENTS

From the standpoint of technical view, such steel-refining agent must satisfy following requirements:

1. It can readily and quickly melt when contacted with the molten steel.
2. As soon as melted, it can quickly spread over the surface of liquid steel to prevent the surface from contacting the atmosphere.
3. When melted by the molten steel it must have a suitable viscosity to spread over the surface of liquid steel.
4. It does not impair properties of steel.
5. If desired, it can readily react with such nonmetallic inclusions in liquid steel as silica, alumina or the like, and remove these impurities.
6. In the case of continuous casting process, it can not only cover the surface of liquid steel but also form a thin film of slag between inside wall of said mold steel and formed slab to prevent rapid cooling of said slab. This is especially important to prevent occurrence of surface cracks of slab having width or more than 1200 mm.
7. It must be inexpensive.

To meet these requirements, the novel steel-refining agent is characterized by the following composition, grain size and chemical and physical properties.

1. Mixing agent:

|                                                           |           |
|-----------------------------------------------------------|-----------|
| Portland cement                                           | 35 to 65% |
| Fluorspar (CAF <sub>2</sub> )                             | 5 to 20%  |
| Chamotte powder                                           | 20 to 40% |
| Soda ash                                                  | 2 to 15%  |
| Source of carbon including graphite powder or coke breeze | 0 to 15%  |
| Borax                                                     | 2 to 15%  |

2. Grading distribution:

The percentage of particles having diameters of less than 0.44 mm. should be more than 50 percent. 3. The refining agent should have a melting point of from 1,000° to 1,300° C., and a viscosity of 1,000 to 10 poises when melted by liquid steel.

15 The purpose of adding borax to the steel-refining agent of this invention is to lower the melting point of said agent to effectively prevent oxidation of the surface of said liquid steel. This is especially desirable for some kinds of steel, for example killed steel.

20 The steel-refining agent of this invention is utilized in the following manner:

It is possible to employ the above agent in bottom pouring process. For example, the novel refining agent in an amount of 0.2 to 2.5 kg. per ton of the molten steel is packed in bags of paper of synthetic resin and these bags are placed in the bottom of a mold or hung therein by means of fine metal wires. When the liquid steel is poured into the mould through a runner brick to come into contact with said bags, the bags are burned to spread the refining agent over the surface of rising liquid steel. A melting point of the steel refining agent ranges from 1,000° to 1,300° C. whereas the temperature of the molten steel is commonly more than 1,300° C., the refining agent will be melted quickly to readily cover the surface of said liquid steel. Since the refining agent has a property of forming slag as flotation of nonmetallic inclusions in liquid steel bath reaches the refining agent slag, said inclusions readily react with a slag layer and adsorbed thereby.

Where the novel steel-refining agent is utilized to cast killed steel ingots by the bottom pouring method it is able to eliminate the use of a coating material which is usually employed to coat inside wall of a mould. Further, nonmetallic inclusions and some streak flaws, such as said inclusion, sand seams and the like are reduced. Following table I shows comparison of the above flaws of low carbon killed steel cast by the prior method and by the novel method in ordinary bottom pouring process.

TABLE I

| 50                                                                | Streak flaws (number of measurement 5) | Agent     |                      |
|-------------------------------------------------------------------|----------------------------------------|-----------|----------------------|
|                                                                   |                                        | Straw ash | Novel refining agent |
| Average number of streak flaws per 100 cm. <sup>2</sup> .....     | 11.3                                   | 4.2       |                      |
| Average length of streak flaws per 100 cm. <sup>2</sup> , mm..... | 10.6                                   | 6.1       |                      |
| Maximum length, mm.....                                           | 5                                      | 4         |                      |

60 A method utilizing the novel steel-refining agent for continuous casting will now be described with reference to the accompanying drawing. As is shown, the liquid steel 3 is poured into a continuous casting mold 2 from a tundish 1 through a long tubular nozzle 4 and when the surface of liquid steel reaches a predetermined level in the mold 2, supply of the novel refining agent is commenced. The relationship between the surface of slag layer formed by the refining agent and the nozzle 4 is as shown in the drawing. The poured liquid steel solidifies to form a cast slab. As the melting point of the steel refining agent is low, as soon as it comes to contact with liquid steel it will be melted to cover the surface of said liquid steel to

TABLE 2

| Percent.....                              | SiO <sub>2</sub> | Al <sub>2</sub> O <sub>3</sub> | CaO   | CaF <sub>2</sub> | Na <sub>2</sub> O | C    | MnO |
|-------------------------------------------|------------------|--------------------------------|-------|------------------|-------------------|------|-----|
| Original component of refining agent..... | 34.8             | 14.4                           | 30.6  | 8.6              | 3.2               | 5.7  |     |
| After melted by liquid steel.....         | 35.7             | 15.7                           | 29.42 | 8.28             | 3.6               | 0.15 | 3.0 |

prevent oxidation thereof by the atmosphere. In this case, it is apparently found that the component of said steel-refining agent changes as shown in table 2.

Due to these components, melting point of the refining agent can form a slag on the surface of said liquid steel which can readily adsorb and remove such nonmetallic contaminants as silica, alumina, etc., in liquid steel. The slag thus formed adheres to the surface of cast slab and then is removed from the mould. As a result it is necessary to constantly add the refining agent into said mold a rate of about 0.3 to 1.2 kg. per ton of liquid steel.

Where the novel steel refining agent is employed for the continuous casting process of billets and blooms, surface defects thereof can be greatly reduced. Accordingly, repairing loss resulting from some surface defects can be improved as shown in tables 3 and 4.

TABLE 3.—WEIGHT RATIO

|                                              |      |                                                |
|----------------------------------------------|------|------------------------------------------------|
| Continuous casting of a 115 x 115 mm. billet | 20   | Repairing loss due to surface defects, percent |
| No refining agent used-----                  | 4. 2 |                                                |
| Used the novel refining agent-----           | 0. 3 |                                                |

TABLE 4.—WEIGHT RATIO

|                                             |      |                                                |
|---------------------------------------------|------|------------------------------------------------|
| Continuous casting of a 1600 x 200 mm. slab | 30   | Repairing loss due to surface defects, percent |
| No refining agent used-----                 | 4. 2 |                                                |
| Used the novel refining agent-----          | 0. 3 |                                                |

Where the novel steel refining agent is not used, the surface of liquid steel killed by aluminum in mold tends to be oxidized by the atmosphere as above described, scum or other slag is formed which caused surface defects. On the contrary, where use is made of the novel refining agent it can not only absorb such scum or slag but also prevent them from being formed. Accordingly, a use of this invention agent can remarkably improved its operability of said continuous casting process and to reduce repairing loss of material surface, while there are many operational difficulties in ordinary continuous casting process of A1-killed steel by reason that said tundish nozzle has tendency to clog.

When slabs having a width or more than 1,200 mm. are moulded by the continuous casting method, longitudinal cracks are formed on the surface of slabs due to thermal stress. However, when the novel steel refining agent is used, the molten refining agent will enter into the gap between the surface of slab and the inside wall of mold to prevent rapid cooling of the slab so that longitudinal cracks due to said heat stress can be effectively prevented. In the continuous casting

of slabs having a width of 1,600 x200 mm. without using the novel refining agent it was noted that longitudinal cracks occurred at a rate of 10 to 30 percent.

Following examples show preferred mixing rate of the novel steel-refining agent.

|                                                           |    |                                                                                      |            |
|-----------------------------------------------------------|----|--------------------------------------------------------------------------------------|------------|
| Example 1: For ordinary steel                             | 10 | Portland cement                                                                      | 44%        |
|                                                           |    | Fluorspar                                                                            | 10%        |
|                                                           |    | Chamotte brick powder                                                                | 32%        |
|                                                           |    | Soda ash                                                                             | 5%         |
|                                                           |    | Coke breeze or graphite powder                                                       | 9%         |
| Example 2: For aluminum killed steel                      | 15 | Portland cement                                                                      | 44%        |
|                                                           |    | Fluorspar                                                                            | 20%        |
|                                                           |    | Chamotte brick powder                                                                | 22%        |
|                                                           |    | Soda ash                                                                             | 5%         |
|                                                           |    | Coke breeze                                                                          | 9%         |
| Example 3: For aluminum killed steel                      | 20 | Portland cement                                                                      | 44%        |
|                                                           |    | Fluorspar 10%                                                                        |            |
|                                                           |    | Chamotte brick powder                                                                | 22%        |
|                                                           |    | Soda ash                                                                             | 5%         |
|                                                           |    | Coke breeze or graphite powder                                                       | 9%         |
|                                                           |    | Borax                                                                                | 10%        |
| Example 4: For stainless steel                            | 25 | Portland cement                                                                      | 44%        |
|                                                           |    | Fluorspar                                                                            | 19%        |
|                                                           |    | Chamotte brick powder                                                                | 24%        |
|                                                           |    | Soda ash                                                                             | 8%         |
|                                                           |    | Coke or graphite powder                                                              | 5%         |
| Example 5: In addition to compounding agent of Example 1; | 30 | Foaming substance (for example, vermiculite, mordenite and foaming synthetic resin). | 0.01 to 5% |

What is claimed is:

1. A steel-refining agent which is composed of 35 to 60 percent of Portland cement, 5 to 20 percent of fluorspar, 20 to 40 percent of Chamotte powder, 2 to 15 percent of soda ash and 2 to 15 percent of carbon source, wherein more than 50 percent of mixing particles have a diameter of less than 0.044 mm.
2. a steel refining agent which is composed of 35 to 60 percent of Portland cement, 5 to 20 percent of fluorspar, 20 to 40 percent of Chamotte powder, 0 to 15 percent of soda ash, 2 to 15 percent of carbon source and 2 to 15 percent of borax, wherein more than 50 percent of mixing particles have a diameter of less than 0.044 mm.
3. The steel-refining agent according to claim 1 wherein said source of carbon is selected from the group which is coke breeze and graphite powder.
4. The steel-refining agent according to claim 2 wherein said source of carbon is selected from the group which is coke breeze and graphite powder.
5. The steel-refining agent according to claim 1 wherein 0.01 to 5 percent of a foaming substance is added to.
6. A steel-refining agent having a chemical composition of  $\text{SiO}_2$  34.8%,  $\text{Al}_2\text{O}_3$  14.4%,  $\text{CaO}$  30.6%,  $\text{CaF}_2$  8.0%,  $\text{Na}_2\text{O}$  3.2% and C 5.7%.